

# UNITED STATES PATENT OFFICE.

ALEXANDER H. TWOMBLY, OF NEW YORK, AND ANDREAS P. LUNDIN, OF BAYSIDE, NEW YORK, AND ROBERT A. MARR, OF NORFOLK, VIRGINIA, ASSIGNEES, BY MESNE ASSIGNMENTS, TO AMERICAN BALSA COMPANY, INC., A CORPORATION OF NEW YORK.

## PROCESS OF TREATING WOOD.

1,396,899.

Specification of Letters Patent. Patented Nov. 15, 1921.

No Drawing.

Application filed January 10, 1917. Serial No. 141,531.

To all whom it may concern:

Be it known that we, ALEXANDER H. TWOMBLY, of New York, N. Y., ANDREAS P. LUNDIN, of Bayside, New York, and ROBERT A. MARR, of Norfolk, Virginia, citizens of the United States, have invented certain new and useful Improvements in Processes of Treating Woods, of which the following is a description in such full and clear terms as will enable any person skilled in the art to which it pertains to make and use the same.

Our invention relates to a process of seasoning wood and at the same time preserving it according to which the wood in any condition, whether green or dried, may be seasoned to any degree of moisture wished, and the wood will be preserved thereafter in this seasoned state regardless of weather conditions to which it may be exposed. The process also affects the removal of constituents in the wood which promote decay and prevents dry rot.

Heretofore it has been proposed to preserve wood by impregnating it with heavy hydrocarbons. Some of these processes have been partially successful, but they have failed of complete success with some kinds of woods. The object of our invention is to provide a process by which any kind of wood may be seasoned to any desired degree of moisture without causing checking or injury to the fibers of the wood and may be preserved in this condition by means of an encysting of its fibers with a substance which renders it substantially waterproof. Our process, furthermore, results in the removal from the wood of those constituents thereof which if allowed to remain in the wood would promote decay.

According to our invention, we first subject the wood to be treated to a preliminary steaming or humidifying process, carried on preferably in a closed retort. The process is begun at a comparatively low temperature and the temperature in the retort is gradually raised by the action of steam heating coils or other heating means. The air within the retort is always maintained in a condition of high humidity, near the point of saturation, vapor or steam jets being discharged into the retort to maintain the proper humidity, water jets being admitted with the steam to this end, if necessary.

During this humidifying process moisture is absorbed by the wood, causing it to swell, dissolving to some extent intercellular matters contained in the wood, such as gums, albumins, sugars, starches and acids. By this treatment, also the cells of the wood are put into better condition to receive and absorb the waterproofing compound without injury, and we believe that the cell walls are rendered softer and more porous and elastic so that in the subsequent treatment of the wood hereinafter described moisture contained in the cells may be driven off without disadvantageous effects on the cell walls or the fibers of the wood. Steaming or humidifying should be begun with the wood at comparatively low temperature and maintained at the low temperature for some length of time in order that the albumins contained in the wood may be dissolved by the moisture absorbed by the wood before the temperature is reached at which albumin coagulates. The temperatures at which the steaming or humidifying process will be carried on and the length of time during which it will be continued vary according to the wood and its condition, and the process continues preferably until moisture has penetrated to the very center of the wood. With an ordinary piece of mahogany wood, 4 x 4 inches in thickness, the process in the steam box may continue for, say five (5) days, the temperature in the retort being graduated progressively from say 100 to 190° F. with the humidity up to 100% during the first part of the time and then gradually lowered after the humidity has penetrated to the center of the wood.

After the wood has been treated as above described it is submerged in a hot bath of a waterproofing compound the boiling point of which is in excess of that of water, the wood being placed in this bath preferably while it is yet warm from the saturation or humidifying process. This waterproofing compound may be of various compositions, but it is preferably composed of a mixture of hydrocarbons, such as asphalt and paraffin, as described in the Broady application for Patent Serial No. 58,232, filed October 27th, 1915, or a mixture of paraffin and naphthalene, such as is described in the Marr Patent No. 1,023,784, or a mixture of paraffin and rosin, such as is described in the Marr Patent

Reissue No. 13,952. We do not, however, wish it to be understood that our invention is limited to the use of these particular substances.

5 The temperature at which this bath is maintained is preferably somewhat in excess of the boiling point of water, and about 220° to 250° F. When the wood is submerged in this hot bath the moisture in the wood passes 10 out from the wood in the form of vapor, carrying with it many of the intercellular constituents of the wood which have been dissolved in the saturation or humidifying process. The vapor passes out, rising in 15 bubbles through the bath, the hydrocarbon mixture enters the cavities of the wood and encysts the cell walls thereof. If a thorough encysting of all the wood cells is desired the process is continued until cessation of the 20 bubbling off of vapor indicates that the moisture has been wholly expelled from the wood, but the process may be continued for as long or as short a time as is desired according to the degree of moisture which it is desired to 25 retain in the wood and according to the thoroughness with which it is desired to encyst the cells.

Preferably we subject the wood in the bath to the process set out in the Broady application, Serial No. 91,109, filed April 14th, 1916, that is to say, we lower the temperature of the bath after the wood has been in it for some time, with the result that as a partial vacuum is produced in the wood by the 30 condensation of vapor within it the vacuum assists capillary action in drawing the hydrocarbon in to the passageways of the wood; and we follow this cooling by a subsequent raising again of the temperature before re- 35 moving the wood from the bath, by means of which the vapor remaining in the wood is expanded again, and a portion of the hydrocarbon which has penetrated is driven out. By means of this cooling and reheating of 40 the bath it is found that a better encysting action is attained, but it will be understood that this is no essential part of our invention.

It will be understood that the duration 45 of this submersion in the bath, like the duration of the steaming or humidifying process, depends upon the character and condition of the wood. Woods that contain a large

percentage of moisture require only a short treatment in order to be thoroughly encysted 55 with the hydrocarbon mixture. Such woods are birch, pine, spruce and balsa. Woods which contain less moisture and are of a denser texture, such as mahogany, oak, etc., require a longer treatment in the steam or 60 humidifying bath and a longer continuance of the lower temperature in said bath since sudden high temperatures have a tendency to cause checking.

Wood treated by this process will be found 65 to be substantially waterproof, and it therefore remains indefinitely in the seasoned state to which it is brought by the process. The process also has the advantages over other seasoning processes that it results in 70 the removal from the wood of intercellular matters, such as albumins, sugars, etc., which by their presence in the wood tend to promote decay, and that the temperatures to which the wood is subjected in this process 75 destroy the spores in the wood which might otherwise cause dry rot, the encysting of the cells preventing subsequent entry of such spores. Furthermore, the process is much shorter than previous seasoning processes. 80

What we claim is:—

The process of treating wood which consists in first humidifying it by exposure to steam the wood being maintained at temperatures above 100° F. and below 212° Fahrenheit, and then subjecting it to a bath of a water-proofing substance heated to a temperature equal to or greater than 212° Fahrenheit. 85

In testimony whereof we have hereunto signed our names in the presence of witnesses.

ALEXANDER H. TWOMBLY.  
ANDREAS P. LUNDIN.  
ROBERT A. MARR.

Witnesses as to Alexander H. Twomby:

ISAAC B. OWENS,  
PATRICK A. BOLGER.

Witnesses as to Andreas P. Lundin:

HARRY W. BROADY,  
WALTER J. KROLMAN.

Witnesses as to signature of Hobert A. Marr:

L. D. STARKS,  
JOHN FARRAS.